

## UNITED STATES PATENT OFFICE.

JOSEPH H. WALLACE, OF STAMFORD, CONNECTICUT, ASSIGNOR TO PINE WASTE PRODUCTS, INC., OF NEW YORK, N. Y., A CORPORATION OF DELAWARE

## PREPARATION OF WOOD FOR PULP MANUFACTURE.

No Drawing.

Application filed August 25, 1920. Serial No. 405,964.

*To all whom it may concern:*

Be it known that I, JOSEPH H. WALLACE, a citizen of the United States, and a resident of Stamford, county of Fairfield, and State of Connecticut, have invented certain new and useful Improvements in Preparation of Wood for Pulp Manufacture, of which the following is a specification.

This invention relates to the treatment of wood, and particularly southern pine in preparation for the manufacture of pulp and for the recovery of high grade products therefrom.

The main objects of the invention, are two-fold, first, to reduce the wood to a size and condition best suited for the manufacture of commercial paper pulp, and second, in the course of such treatment to recover valuable products carried by the wood.

At the present time one of the most available sources of wood for pulp purposes is the yellow pine of our southern forests, including what is known as the long and the short leaf, Cuban and loblolly. Other available sources are the balsams, the various tamaracks and Douglas fir. These pines, as well known, possess long grained fibres of a superior character for paper making and also carry a large proportion of valuable turpentine and resinous compounds. This high content of turpentine and resin has made the treatment of these woods for pulp purposes particularly difficult. In the alkali processes, too much of the alkali is consumed by combination with the resins; and the digester liquor is cumbered with great amounts of resins and resin soaps. The paper maker wants some resin present, but not too much; and he does not desire highly acid resins. Further, the material is irregular as regards its composition, some chips being highly resinous while others are not, which renders operation irregular. For these reasons the pines mentioned, in spite of their high grade fiber, have not been much used.

In the present invention, I obviate these difficulties by submitting the wood to what may be called a partial extraction treatment, removing some but not all of the resins and terpenes. I aim to take out a substantial quantity of the total extractable matter, while leaving a substantial quantity behind. From the paper maker's standpoint this has

the advantage of providing an open textured, pervious chip containing some, but not much resin and having the resin therein substantially uniformly distributed; while it has further very great advantages from the view point of the quality of the extracted matter.

Southern pine contains many and varied substances of the general nature of terpenes and resins; and it is common to submit it to extraction to regain these. Many methods have been proposed, and many hundreds of patents dealing with this problem have been issued. Most of these treat finely divided wood with some solvent such as gasolene, benzol, benzine, naphtha, etc.; others suggest a mild treatment with solutions of alkalis to saponify the resin and render it water-soluble without attacking the remainder of the wood. Solvent methods have advanced the farthest along the road toward successful commercial exploitation, but none of these has yet attained complete success. This is for various reasons, one being that the effort is to do too much; to get as great a quantity of extractive as possible. The wood is comminuted in order to aid extraction; and this ruins the residue for the paper making process. Another is that in securing a large total yield of extractive, the quality of the product is low.

The highest grade rosin or colophony made is procured from clean gum turpentine. The pine wood itself contains this same material; but it also contains very many other things; and with any long continued and exhaustive extraction, these other things are also extracted and reduce the grade of rosin produced very much.

I have found that if the wood be extracted with a solvent, the operation really takes place in two phases; a first stage where extraction is rapid and the extract is of high grade, and a second stage where extraction becomes very slow and the products dissolved are largely of gummy, viscous and amorphous nature. Naturally the two stages shade into each other to a certain extent; but nevertheless, there is a tolerably abrupt change. By confining the extraction to the first stage, high grade turpentine, pine oil and rosin are produced; and in practice it is worth while, where an exhaustive extrac-

tion is wanted, to secure the two extracts separately. If however chips for paper making are wanted, it is better to confine the operation to the one stage, leaving residual 5 resins and terpenes in the wood for the pulp mill to deal with. As stated, the presence of a certain amount of these bodies is desirable for pulp mill purposes in any event.

In the practice of my invention the coniferous wood is reduced to pulp mill size,—that is long fibred chips of a size best answering the requirements of the paper manufacturer. These mill size chips may average from  $\frac{5}{8}$  to  $\frac{7}{8}$  of an inch in length,  $\frac{1}{2}$  to  $1\frac{1}{4}$  inches in width and  $\frac{1}{8}$  to  $\frac{3}{16}$  inches in thickness.

These long fibred mill size chips are charged into what I have termed an "extractor" and there treated with a solvent 10 preferably like the natural solvent disclosed by Clope Patent No. 1,144,171 June 22, 1915. As an object of the present invention is to obtain high grade extractives by a partial extraction, this solvent is here particularly 15 useful as it imparts nothing foreign to the extract. This solvent may be applied either in the form of a liquid or vapor. At the present time, I prefer to use the liquid and in a moderately heated condition. This liquid 20 is caused to percolate or circulate through and around the body of chips and in its passage it extracts the resin, turpentine, pine oil and also a fresh supply of the natural solvent. These products are suitably 25 collected and separated, usually by distillation, in which case, the turpentine passes off at and around 160 degrees C., the solvent between about 160 and 180 degrees C., and the pine oil at and above approximately 180 30 degrees C., leaving the resin as a residue.

This treatment is not continued, as in Clope, to the point where a substantially complete extraction is effected, but on the contrary it is discontinued after the point of 35 maximum efficiency is reached. This point may be determined by tests, and depends upon a number of different factors. The extraction is more rapid at the beginning, tapering off in volume as the operation proceeds, and at the point where it is no longer 40 economically profitable the operation is discontinued. In different runs which I have made the extraction has been carried on for periods ranging from about  $\frac{1}{2}$  to 2 hours as 45 against 4 to 6 hours needed for the usual process.

A convenient method of determining the extraction period is to plot extraction curves 50 showing the rate of extraction in intervals of time. These curves show a rapid extraction for the first short interval of time, and an abrupt change in the direction of the curve at the end of this first extraction period. The approximate location of the commercially 55 efficient point for the discontinu-

ance of the extraction is therefore indicated by this relatively abrupt change in the extraction curve. This point will vary moderately however, with changes in the market value of the products and labor charges and other elements entering into the cost of production. For instance, at a time when turpentine and rosin have a high market value, the commercially efficient period of treatment will be longer than at a time when 60 these products are at low market value. It is a commercial question between more and lower grade extract and less extract of higher grade. In all events, however, the extraction is continued to a point where the 65 chips are free of the turpentine and resinous constituents to such an extent that they may be economically handled in the usual paper making processes. Ordinarily this point is reached where about 30 per cent of the total 70 extractable matter is left.

At the end of the extraction treatment, steam or other agent may be passed through the chips to clear them of the free solvent.

The apparatus necessary for the partial extraction described, is relatively simple and may be made in portable form so that it is possible to carry out this new process in the woods, or in other words at the source. No chemicals are required other than the natural solvent, and this as above described, is produced as needed at the field plant.

After treatment nothing is left with the cellulose but those materials which are readily removed by the pulping process. The 80 chips are in a porous condition and therefore easily reduced to pulp, and what is quite important to the paper manufacturer, have a substantially uniform and constant moisture content. This enables the pulp maker to deal with the chips with greater 85 certainty and less experimentation than has been possible heretofore where the moisture content varies greatly.

The suspension of the extraction treatment 90 after the removal of that portion of the resinous and other materials which can be obtained with the minimum of time and effort and the maximum of efficiency, keeps the cost of extraction at a commercially economical point, and furthermore, results in the production of superior grades of the resin and other constituents. This is because 95 superior products are extracted during the early part of the treatment, that is in the 100 period of maximum extraction efficiency. I attribute this partly to the fact that the natural resins occurring in the pine in time undergo oxidation and other injurious transformations subsequent to their formation in the tree, which transformation products are 105 inferior to the virgin gum. This is particularly true of the resins in stumps and dead trees, or in other words, "lightwood," a material which is most available for solvent 110

treatment. These inferior resins are less readily acted upon by the natural solvent, and a short treatment therewith, results in the removal of a lesser amount of the same.

- 5 Another important point of my invention arises, from the fact that any long exposure of the resins, especially rosin, to heat and to contact with metals, particularly iron, produces decomposition resulting in diminution 10 in the value of the resins. The reduced extraction of my invention involves a substantially lessened exposure of the resin to heat and contact with the metal of the apparatus so that the resin produced is for this reason 15 also of a superior quality.

From the foregoing, it will be seen that my invention furnishes to the pulp manufacturer a long fibred mill size chip ready for the pulping process and which is porous 20 and has a substantially standardized moisture and resin content, and therefore, best fulfills requirements of pulp making. Furthermore, the preparatory work on these chips can be commercially and inexpensively 25 carried out directly at the source. It is also apparent that the process is an economical one, commercially practicable, and that by it are obtained high grade extraction products.

- 30 By stopping the extraction process at the point of maximum efficiency or commercial economy, the by-products can be made to pay for the chips, and the chips freed of the greater part of the turpentine and resinous 35 constituents provide a superior material for pulp purposes. All the operations described may be readily carried on in the woods, and the apparatus necessary is not expensive, or complicated or cumbersome because the operations are carried on at low 40 pressure and low temperature. The distillation for the separation of the more volatile constituents from the resin may be carried on in the field or at any convenient 45 point, but at any rate, the resin is usually removed at the field plant.

On the other hand, if the partially extracted 50 chips are to be shipped some distance the moisture content may be reduced by a suitable drying process to approximately 12 to 20 per cent, so that the chips will not give up or take on moisture in transit and will be received at the paper mill with a known moisture content, and can be treated 55 accordingly.

The partially extracted chips are subjected to a "cooking" process at the pulp mill to reduce them to the cellulose condition necessary for pulp manufacture. Usually this is accomplished by disintegrating chips 60 in digesters by means of a hot solution of chemicals such as caustic alkali or acid 65 terpenes as were not removed in the partial extraction treatment of the chips may be

recovered, in a large measure, in this latter stage of the operations from the waste gases of the digester.

In an application, Serial No. 405,963, filed herewith, I have described and claimed a process similar to that disclosed herein for recovering extracts from resinous woods, and in another application, Serial No. 405,965, also filed herewith, I am claiming such pulp mill chips as may be made by means of the present invention.

What I claim is:

1. The process of producing long-fibred relatively porous pulp mill chips having materially less resinous matter than that normal to the wood, said resinous matter being distributed substantially uniformly therethrough, which comprises reducing resinous coniferous wood to pulp mill-size chips, subjecting the same to a solvent throughout that period where the action of the solvent is most rapid and the rate of extraction is highest, and discontinuing such extractive treatment at or about the point where there is an abrupt reduction in the rate of extraction of matters soluble in said solvent and while there yet remains in said chips a substantial amount of matters soluble in said solvent.

2. The process of producing a material for pulp mills which comprises treating resinous coniferous pulp mill chips with a solvent throughout that period where the solvent is most active and the rate of extraction is highest, and discontinuing such extractive treatment at or about the time the rate of extraction is abruptly reduced and while there yet remains in said chips a substantial amount of matters soluble in said solvent.

3. The process of treating resinous coniferous wood to remove the extractives of greater value and to leave the wood in open porous texture with a substantial quantity of resinous matter less than that normal to the wood distributed substantially uniformly therethrough, which comprises subjecting the wood to the action of a hot solvent throughout a period of time which is relatively short as compared to that necessary for complete extraction of the wood by said solvent and discontinuing such extractive treatment substantially at the end of the period where the extraction rate is highest and substantially at that point where only the lighter extractives have been removed; said wood still retaining a substantial amount of matters soluble in said solvent.

4. The herein disclosed process which comprises only partially extracting pulp mill chips with a solvent and then subjecting said partially extracted chips to a pulping treatment in which the residue of the extractives in the partially extracted chips is removed.

5. The herein disclosed process which comprises only partially extracting pulp mill chips with a solvent and then subjecting said partially extracted chips to a pulping treatment in which the residue of the extractives in the partially extracted chips is removed, including the recovery during such pulping treatment of such volatile terpenes as were not extracted during the first operation above. 10
6. In witness whereof, I have hereunto set my hand this 23d day of August, 1920.

JOSEPH H. WALLACE.